

# UNITED STATES PATENT OFFICE.

JAMES H. STEBBINS, JR., OF NEW YORK, N. Y.

## DYEING BLUE COLORS UPON TEXTILE FABRICS.

SPECIFICATION forming part of Letters Patent No. 255,349, dated March 21, 1882.

Application filed February 1, 1882. (Specimens.)

*To all whom it may concern:*

Be it known that I, JAMES H. STEBBINS, Jr., a citizen of the United States, residing at New York, in the county and State of New York, 5 have invented new and useful Improvements in Producing a Blue Color in or upon a Textile Fiber or Fabrics, of which the following is a specification.

This invention relates to the production of 10 a blue color produced by the action of diethyl-paraphenylenediamine chloride upon an alkaline solution of alpha-naphthol in the presence of an oxidizing agent in or upon a textile fiber or fabrics.

15 In carrying out this invention I proceed as follows: For printing purposes I prepare or impregnate the cotton cloth or calico to be printed with an aqueous solution of the soda salt of alpha-naphthol, and then dry with dry heat at 20 a temperature of about 150° Fahrenheit. This prepared cloth is then printed with a mixture of nitroso-diethylaniline chloride and an alkaline solution of grape-sugar which has been made into a thickening or paste with starch, 25 or otherwise, in the usual manner. After printing, the blue color is developed by steaming in the usual manner, and then the printed calico is to be washed and cleared. Care should be taken that so much of the alkaline solution of 30 grape-sugar is mixed with the nitroso-diethylaniline chloride as to completely reduce it into its base.

Another method for printing cotton cloth or calico is the following: I prepare or impregnate the cotton cloth or calico to be printed with an alkaline solution of grape-sugar, and then dry it with dry heat at a temperature of about 200° Fahrenheit. This prepared cloth is then printed with a printing-color suitable 35 for calico-printing, which may be prepared by mixing about ten pounds of nitroso-diethylaniline chloride, fourteen pounds of alpha-naphthol, fourteen pounds of caustic-soda solution, (1.29 specific gravity,) and with sufficient water 40 to dissolve the mixture, and then with starch-paste or other suitable thickening the color thus prepared is ready for printing the cloth. 45

Another method for printing cotton cloth or calico is the following: I take ten pounds of nitroso-diethylaniline chloride and dissolve 50 it in one hundred pounds of water, then add fifteen pounds of zinc-dust, and heat the mixture, under constant stirring, to about 60° centigrade, by which the nitroso compound is to be reduced to diethylparaphenylenediamine 55 chloride. The zinc-dust is then separated by filtering and the solution allowed to cool. To this I add an aqueous solution of about twenty-seven pounds of soda salt of alpha-naphthol and sufficient starch-paste or other suitable 60 thickening to make a suitable printing-color. The color thus prepared is ready for use and ought to be employed for printing without much delay, as upon standing the color is liable to decompose. With this prepared printing-color I impregnate or print the cloth or calico to be printed, and then steam in the usual way. The so prepared cloth or calico is then passed through a hot aqueous solution of bichromate of potash, by which the blue color is 65 more fully developed. The so printed cloth is then washed, soaped, and cleared in the usual way. By this method woven fabrics of wool, and of cotton and wool mixed, and also woolen yarn, can be prepared and printed and the blue 70 color developed thereon.

75 What I claim as new, and desire to secure by Letters Patent, is—

As a new article of manufacture, textile fiber, 80 yarn, or cloth, whether knit or woven, having the herein-described color developed within or upon the same by the reaction in or upon the fiber of nitroso-diethylaniline chloride and the soda salt of alpha-naphthol in the presence of an oxidizing agent, substantially as set forth, 85 or by any other means which will produce a like result.

In testimony whereof I have hereunto set my hand and seal in the presence of two subscribing witnesses.

JAMES H. STEBBINS, JR. [I. S.]

Witnesses:

W. HAUFF,  
J. A. RUTHERFORD.